

Oct. 6, 1925.

1,556,200

F. C. BRANDENBURG

SHOVEL

Filed Jan. 17, 1921



Patented Oct. 6, 1925.

1,556,200

# UNITED STATES PATENT OFFICE.

FRANCIS C. BRANDENBURG, OF PIQUA, OHIO, ASSIGNOR TO THE WOOD SHOVEL AND TOOL COMPANY, OF PIQUA, OHIO, A CORPORATION OF OHIO.

## SHOVEL.

Application filed January 17, 1921. Serial No. 437,763.

To all whom it may concern:

Be it known that I, FRANCIS C. BRANDENBURG, a citizen of the United States, residing at Piqua, in the county of Miami and 5 State of Ohio, have invented a new and useful Improvement in Shovels; of which the following is a specification.

My invention relates to shovels, as articles of manufacture, in which the cutting edge, 10 i. e., the edge that must cut or slide under the material to be lifted by the shovel, is stiffened and held straight by a slight bend or camber a short distance from and parallel to the cutting edge; and in which the shovel 15 is hardened by heat-treatment.

In the accompanying drawing, Figure 1 is a perspective view of a shovel embodying my present invention and Figure 2 is a longitudinal sectional view thereof.

20 Outwardly this shovel resembles many others, but it differs from them in that the structure of the metal composing it contributes to the maintenance of a predetermined form, where in other shovels, especially 25 heat-treated shovels, the desired form, if it is maintained at all, is maintained by a sort of balance or equilibrium of opposing strains, each tending to distort the metal.

Heat-treating shovels is not new; neither 30 is it new to provide heat-treated shovels with the camber. But certain difficulties have been encountered by those who produce heat-treated cambered shovels, the principal of which is that such shovels do not retain 35 their shape. Sooner or later they become distorted. It is not practicable, obviously, to bend the shovel after it is heat-treated. Even if the metal is not too hard to permit of its being bent, bending it after it has been 40 heat-treated sets up internal and opposing stresses in the metal, which either immediately or eventually distort the shovel, so that the edge becomes crooked and its usefulness much impaired. Neither is it practicable 45 to make the bend before the heat-treating is done, because of the tendency of the metal to warp and become distorted during the heat-treatment. This has been tried, and is being done by others, and it is to overcome 50 the difficulties encountered by those who use that method that I have devised my new method. As is well known, there is always more or less certainty that sheet metal will warp during heat-treatment, and in a case 55 such as forming the camber in a shovel, this

condition is much aggravated. The excessive tendency of the camber to warp during heat-treatment is due to the slightness of the bend in the metal. Where a considerable or very sharp bend is made in sheet 60 metal, a certain disruption of the bonds uniting the metallic crystals occurs, which eliminates to a considerable extent, if not wholly, the tendency for the metal to return to its former shape. In other words, 65 the metal is strained beyond its elastic limit and becomes "set" in its new position. In cambering a shovel the metal is bent so slightly that it is not strained to its elastic limit, or at least not to the extent necessary 70 to eliminate all tendency to return to its former shape, and the shovel is certain to warp when the metal is heated. At present this difficulty is being met by other shovel makers by straightening the shovels with a 75 hammer after they are heat-treated.

To overcome the difficulties described I have developed a method for simultaneously cambering and heat-treating shovels. Briefly, this method consists in providing a 80 pair of forming dies between which the lower end of a heated shovel may be clamped and the desired camber formed therein. This device is immersed in a 85 quenching liquid and means provided for operating the dies while immersed. The shovel is heated to a degree above the critical temperature of the metal, then plunged into the quenching liquid and clamped between the dies before the metal has had 90 time to cool below its critical temperature. The metal is very malleable when heated above its critical temperature, and its crystals, also the bonds uniting them, readily 95 adapt themselves to their new positions, so that when the metal is cooled the structural arrangement of the metal, that is, the crystalline formation of the metal is such as tends to maintain the position it was forced 100 by the dies to assume. It may be said that the crystalline structure is inert; i. e., the bonds uniting the crystals tend to hold the crystals in the position they occupied while the shovel was between the dies, and the metal is therefore devoid of tendency to assume another form. The metal not only 105 has no tendency to change its shape, but it is endowed with power to resist extraneous strains tending to distort it.

My shovels are thus distinguished in a 110

very important and definite way from those which are allowed to warp during heat-treatment and afterward straightened with a hammer or by other means. They are unwarped, not dewarped. Straightening the hardened metal after it has warped simply sets up opposing strains which, though for the time being may balance one another and hold the metal straight, eventually become unbalanced and distortion of the metal follows. If this does not occur through the ordinary "seasoning" process which the metal undergoes, it is brought about by strains occurring in the ordinary use of the shovel, or because of the wearing away of parts of the metal which constitute elements in the artificially created equilibrium of strains. In my shovel the metal is given its form while hot, the constituents of the metal being then in a state of repose, and the metal is hardened with the same heat. Therefore, the crystalline structure is in harmony with the form of the shovel. The metal is not only free from strains tending to distort it, but being inert its entire mechanical strength is available for resistance to external strains tending to distort it. Moreover, since the constituents of the metal are in a state of repose, my shovels retain their shape as they wear out.

In addition to the obvious advantage of keeping the cutting edge straight, so that

when the shovel is used, say to lift ashes or coal, it bears on the ground or floor over the entire width of the shovel, the camber is also advantageous in that it insures a narrow contact with the floor, which contact is certain to be at the cutting edge. 35

In an application filed concurrently with the present one, Serial No. 437,764 I have described my method in detail and also apparatus for putting the method into effect. So it is deemed unnecessary to repeat the description here. 40

Having fully described my new article of manufacture, what I claim is as follows:

1. A heat-treated steel shovel having a straight cutting edge, the heat-treated metal in said shovel being substantially free from 50 stresses produced by cold working.

2. A heat-treated steel shovel having a straight cutting edge and a camber near and parallel to said edge, the heat-treated metal composing the shovel being substantially 55 free from stresses produced by cold working.

3. A heat-treated steel shovel having a straight, single ply, cutting edge, the heat-treated metal in said shovel being substantially free from 60 stresses produced by cold working.

4. A heat-treatment-hardened steel shovel having a straight cutting edge, the hardened metal in said shovel being substantially free from stresses produced by cold working.

FRANCIS C. BRANDENBURG.